

Patented July 2, 1929.

1,719,464

# UNITED STATES PATENT OFFICE.

WILLIAM HOWARD COLE, OF PARIS, FRANCE.

## PROOFING OF IRON AND STEEL AGAINST RUST.

No Drawing. Application filed March 11, 1929, Serial No. 346,249, and in Great Britain January 29, 1929.

This invention is an improvement in or modification of the inventions described and claimed in my applications for Letters Patent Ser. Nos. 171,730 and 171,731. In the 5 said specifications I have described new processes for proofing iron and steel against rust consisting in effecting a deposit on the articles proofed by treating them under the conditions described with a special solution 10 of phosphates of aluminium, zinc, iron and chromium. The present invention relates to a selection of conditions and proportions included in my said prior specifications, but which I have found, upon further experiment, to give the best possible result.

According to my invention, I provide a process for the proofing of iron and steel against rust, substantially as claimed in specifications Ser. No. 171,730, in which iron, 20 zinc, chromium and aluminium are used.

To make the processing solution I use:

Iron filings (clean and free from scale), zinc powder, aluminium powder, and chromium powder.

25 It is a feature of the present invention that these are dissolved separately at a temperature not over 90° C. in a solution of phosphoric acid 45° Bé. diluted with water to 22° Bé. until the said metallic phosphatic 30 solutions are each of a density of 36° Bé.

In dissolving, the temperature should be retained as constant as possible during the whole time of dissolution but in no instance should it go above 90° C. and during said 35 period of dissolution the containers should be covered in order to save any loss from evaporation.

These four solutions at the said 36° Bé. are then mixed together in the following 40 proportions:

1 part aluminium solution, 5 parts zinc solution, 5 parts iron solution,  $\frac{1}{2}$  part chromium solution.

In place of chromium powder, chromium 45 oxide may be used for economical reasons as being less expensive, takes less time for dissolution and, further, I find no material difference in the results.

To this mixture is then added a solution 50 or mixture of the following ingredients and in the proportion hereinafter described:

25 grammes bichromate of potassium, 70 grammes neutral chromate of potassium, 25 grammes monobasic phosphate of ammonium, 5 grammes naphthalene.

This mixture is dissolved or suspended in

$\frac{1}{2}$  litre of water (distilled water is preferable).

4 cubic centimetres of this solution or suspension are then added to each litre of the 60 phosphate solution of the four above-mentioned metals.

This solution I now term the stock liquor.

The quantities of the above-mentioned ingredients are given in grammes, but they 65 may be assembled in any unit or quantity so long as these proportions are used.

Although only a small quantity of the mixture of ingredients is used, nevertheless I find it is most important and has a most 70 singular effect and influence on the results of the operation.

The addition of these ingredients has for its purpose to obtain the full value of the combination of metals. In my view they 75 act as follows:—

Bichromate of potassium gives cementation effect of the combined precipitated mass when it attacks the iron or steel surfaces.

Neutral chromate of potassium creates a 80 special affinity between the four metals after they have been dissolved. The use of chromium gave a considerable amount of trouble in uniting with the other metals in solution after they were dissolved, and I 85 found that this ingredient had a decided cohesive influence, as between the chromium and the other metals.

Monobasic phosphate of ammonium holds for an instant the final combination of the 90 precipitants until all of the metals have been thrown down.

Naphthalene is used principally in that it aids in the union of the combined precipitants on to the surface of the articles 95 treated.

The stock liquor may be used direct for processing, after being diluted to about 3° Bé. or it may be evaporated down to salts or a compound (as I call it), for ease in 100 handling or transportation.

In evaporating over heat, care must be taken that it is never done above a temperature over 90° C. and that care must be taken so as not to permit of its burning. It is 105 advisable that constant stirring be done during evaporation.

The salts or compound is ready for processing by simply mixing with water to about 3° Bé.

For processing, the solution at about 3° Bé. is placed in any suitable tank, prefer-

ably closed, so as to permit of a pressure within, and heated to a temperature around the boiling point but above 90° C. and preferably about 95° C.

- 5 It will be noted that the processing operation is effected at a temperature higher than that at which the metals are dissolved. It appears as if a certain amount of acid became free or active under the higher temperature of processing and this appears to be necessary for a successful operation in the process.

10 Into this are placed the iron or steel articles (preferably in a suitable container or cage) and allowed to remain from 1 to 1½ hours. The temperature should be constant during the operation.

15 There should preferably be a constant change of contact of the articles being treated during the processing operation.

20 Before processing, articles to be treated should be as clean as possible and free from rust, scale and dirt.

25 It is advisable to have sufficient solution in excess in the processing tank. It is recommended that this be at least 1½ to 2 times the quantity necessary, although a greater amount does not harm.

30 Both before and after processing, the solution in the tank should be measured, so that the solution may be properly adjusted for the next operation of processing. Sufficient water is added to take the place of that evaporated during the process and then sufficient stock liquor is also added to bring the solution to the original operating specific gravity.

35 It will be understood that good results can be obtained whilst departing from the quantities of metals and other ingredients, varying the stated temperatures and densities, but I have found that the best results are obtained by observing the conditions herein described, which are selected from, and in 40 some respects modifications of, my specifications Ser. No. 171,730.

45 What I claim and desire to secure by Letters Patent is:—

50 1. The improvement in proofing of iron and steel against rust, which consists in preparing the processing solution from the four metals, iron, zinc, aluminium and

chromium, by dissolving each of the metals or the oxide of chromium separately at a temperature not over 90° C. in a solution of phosphoric acid of 45° Bé. diluted with water to 22° Bé. until the said metallic phosphatic solutions are each of a density of 36° Bé., mixing these solutions together in the proportions: 1. part aluminium solution, 5 parts zinc solution, 5 parts iron solution and ½ part chromium solution.

55 2. The improvement in proofing of iron and steel against rust, which consists in preparing the processing solution as claimed in claim 1, and adding to it a small quantity of a solution or suspension containing bichromate of potassium, neutral chromate of potassium, monobasic phosphate of ammonium and naphthalene in the proportions 60 70 25 grammes bichromate of potassium, 70 grammes neutral chromate of potassium, 25 grammes monobasic phosphate of ammonium, and 5 grammes of naphthalene.

75 3. The improvement in the process of proofing iron and steel against rust comprising the preparing of a processing solution of iron, zinc, aluminium and chromium dissolved separately in a solution of phosphoric acid and then combining the same, diluting 80 this solution with water to about 3 degrees Bé. and then treating the articles to be proofed with this resulting solution at about 95 degrees C. which temperature is higher than that at which the metals were dissolved 85 in solution.

4. In combination in a compound for rust-proofing of metal, comprising a solution of phosphoric acid having one part aluminium, five parts zinc, five parts iron and one-half 90 part chromium.

5. In combination in a compound for rust-proofing of metal, comprising a solution of phosphoric acid having one part aluminium, five parts zinc, five parts iron and one-half 95 part chromium, and a second solution comprising 25 grammes bichromate of potassium, 70 grammes neutral chromate of potassium, 25 grammes monobasic phosphate of ammonium and 5 grammes of naphthalene. 100

In testimony whereof, I affix my signature.

WILLIAM HOWARD COLE.